

June 7, 1960

M. C. HOLLAND

2,939,202

SYNTHETIC POLYMER TEXTILE FILAMENT

Filed Dec. 31, 1959

2 Sheets-Sheet 1



*James C. Earle*

ATTORNEY

June 7, 1960

M. C. HOLLAND

2,939,202

SYNTHETIC POLYMER TEXTILE FILAMENT

Filed Dec. 31, 1959

2 Sheets-Sheet 2



2,939,202

## SYNTHETIC POLYMER TEXTILE FILAMENT

Marlin C. Holland, Wilmington, Del., assignor to E. I. du Pont de Nemours and Company, Wilmington, Del., a corporation of Delaware

Filed Dec. 31, 1959, Ser. No. 863,189

8 Claims. (Cl. 28—82)

This invention relates to novel synthetic fibers and filaments having a unique combination of improved optical and physical properties.

Fibers having various cross-sectional shapes have been prepared to provide textile materials having certain desirable properties. For example, fibers having a Y-shape cross section have been used in fabrics to provide bulk. Similarly, fibers have been made with other cross sections, e.g., ribbon, dumbbell or dogbone shape and cruciform, to provide improvements in other textile properties. Fibers having a trilobal configuration which provide unique luster highlight in addition to other desirable properties are described in my copending application Serial No. 822,514, filed June 24, 1959, which is a continuation-in-part of my application Serial No. 748,447, filed July 14, 1958, now abandoned. The filaments described in my copending application have three symmetrical lobes, with each lobe having essentially straight side portions extending outwardly and tangent to an arcuate portion at each end. I have now discovered that this unique luster highlight is also found in other trilobal filaments having side portions which are convex. In addition to the unique optical properties, the fibers having convex side portions provide other improved properties which are particularly desirable in flat textile fabrics.

Accordingly, it is an object of this invention to provide fibers and filaments having a trilobal cross section which are particularly adapted for use in flat textile fabrics. A more specific object of this invention is to provide novel synthetic fibers and filaments which, when incorporated in apparel fabrics, exhibit a unique combination of luster highlight, drapability, resistance to soiling, covering power, and wrinkle resistance. Other objects will appear hereinafter.

The objects of this invention are accomplished by providing novel filaments and fibers prepared from synthetic polymers having a cross-sectional shape consisting of three convex sides and three arcuate terminal portions. The convex sides may be made up of two straight portions which join the curved portion to the adjacent arcuate tips. The tips of the three terminal portions of the cross section of the filaments define a circle having its center equidistant from the tips. The cross section may be divided into three portions, each including a tip, which are essentially symmetrical in shape. Filaments of the present invention are members of the tribrachiate family and may be defined by any three of five parameters whose interrelation is given by the two equations set forth in my aforementioned copending application. It must be noted, however, that it is only by maintaining the parameters describing the cross-sectional shape within certain limits, to be more fully defined later herein, that the combination of properties previously mentioned are obtained.

Throughout the specification and claims, the terms "filaments" and "fibers" will be used interchangeably in their usual and accepted meaning. By the term "luster

"highlight" is meant the frequency and the degree of concentration (in area) of the high intensity light reflected from a small area of a yarn or textile material relative to the average of the total amount of light reflected from

5 a portion of the same yarn or textile material which includes the small area. By the term "soiling resistance" is meant the apparent resistance of a textile material to visible soil which may be independent of the soiling which may actually occur.

10 The present invention will be more fully understood by reference to the following detailed description and the accompanying drawings in which:

Figures 1 and 2 are enlarged representations of cross sections of the filaments of this invention;

15 Figures 3 and 4 are graphs showing the area in which the parameters defining the cross section of the filaments of this invention appear; and

Figure 5 is an enlarged view of a spinneret orifice which may be used in spinning the filaments of the present invention.

20 Referring now to Figs. 1 and 2, the cross-sectional shapes of the filaments of this invention are defined by the following parameters:

(1) The ratio of the tip radius  $r_1$  to the radius  $R$  of a

25 circle  $a$  having a center  $c$  circumscribed about the tips  $b$ ;

(2) The arm angle  $A$  formed by extending a line tangent to both the convex side  $d$  and the arc generated by the tip radius  $r_1$  (when there is a straight portion joining the tip and convex side, this straight portion will be a common tangent to both the tip circle and the convex side and will determine the angle  $A$ . When there is no straight portion, the convex side and the tip circle will have a common tangent which will determine the angle  $A$ ); and

30 (3) The ratio of the radius  $R$  to the radius  $R^1$  of a circle having center  $c$  inscribed within the cross section which will be referred to as the modification ratio  $M$ .

35 As previously indicated, the equations set forth in my copending application express the interrelation of the

40 aforementioned parameters. In all of the filaments of the present invention, the arm angle  $A$  is greater than 60°. In general, the modification ratio  $M$  is from about 1.1 to about 1.63, the tip radius ratio

$$\frac{r_1}{R}$$

45 is from about zero to about 0.71, and the arm angle  $A$  is from about 70° to 150°. However, not all combinations of the aforementioned parameters will provide filaments having the improved properties heretofore described. It is only filaments having combinations of parameters selected from the cross-hatched areas of Figs. 3 and 4 which provide the new and unusual properties. It will be noted that the areas shown on the graphs are not regular geometrical figures as one might expect. If a three-dimensional plot were made incorporating the points on the graphs, it would appear as a volume with those filaments exhibiting maximum luster being found at the position where angle  $A$  is about 110°,

$$\frac{r_1}{R}$$

50 60 65 70 is about 0.3, and  $M$  is about 1.28.

It is indeed surprising that the filaments of the present invention exhibit a unique luster highlight since sparkle and glitter have heretofore been thought to be attributable to the presence of relatively large, flat surface areas along the fiber axis. It is also surprising that the filaments of the present invention exhibit a much higher resistance to wrinkling and soiling than fibers having either a triangular

or Y-shape cross section while at the same time exhibiting the luster highlight property.

In preparing the filaments of the present invention, a spinneret having orifices of a configuration similar to that shown in Fig. 5 may be used. Spinning conditions must, of course, be varied, depending on the particular synthetic polymer being spun. Certain adjustments in the dimensions of the orifices, the viscosity of the polymer, the melt temperature, and the quenching conditions may be necessary in order to produce filaments having parameters within the limits previously described. Conditions should be controlled to give filaments which have a substantially uniform cross-sectional shape along their length.

Although the shape of the filaments must remain within the limits previously described, slight variations in the parameters may occur along the length of the filament or from filament-to-filament in a bundle without adversely affecting their unique properties. In addition, the cross sections may not be perfectly symmetrical.

The denier of the filaments may vary within wide limits. Deniers in the range from 1 to 35 are usually preferred; however, deniers of 250 or higher may be utilized, depending on the end use of the textile material being prepared.

This invention will be more fully described in the following examples which are illustrative and in which parts and percentages are by weight unless otherwise specified. The various tests used to illustrate the improved properties of the filaments of this invention are described in detail in the examples.

#### EXAMPLE I

A sample of polyester filaments was prepared from a copolymer of polyethylene terephthalate modified with 2 mol percent sodium-2,5-di(carbomethoxy)benzene sulfonate. The polymer had a relative viscosity of 22.3 as measured in a 10% solution of the polymer in a mixture of 10 parts of phenol and 7 parts of 2,4,6-dichlorophenol at 25° C. The polymer contained 0.3% titanium dioxide by weight.

The polymer was melt spun at 296° C. through a stainless steel spinneret having 70 capillaries. Each spinneret orifice was triangular in shape with each side being 12 mils in length. The filaments, upon being extruded from the spinneret, were quenched in cross-flowing air having a velocity of 65 feet per minute and a temperature of 70° C. They were wound up as a 50-filament bundle at a windup speed of 1500 yards per minute. The total denier of the spun yarn was 152. The spun yarn was then drawn at a temperature of 107° C., using a one-quarter inch diameter snubbing pin, a draw ratio of 2.14, and a windup speed of 604 yards per minute. The drawn yarn was found to have a total denier of 70.3, a tenacity of 3 grams per denier, and a break elongation of 24.2%.

A taffeta fabric was woven from the yarn. In weaving, a twist of five 2 turns per inch was used in the warp and zero twist in the filling. The loom construction was 100 ends × 80 picks. After weaving, the fabric was scoured at the boil in an aqueous medium in a relaxed condition and then dried. The fabric was then heat set for one minute at 390° F. and then finished. The fabric sample is identified as sample F-1.

For comparative purposes, similar fabrics were prepared from two other polyester yarns, each differing from sample F-1 only with respect to the cross-sectional configuration of the fibers used in the fabric. Sample F-2 was woven from round filaments and sample F-3 was woven from filaments having a trilobal configuration with parameters described in Table 1. Each of the fabrics were tested for covering power, luster highlight, and soil resistance in accordance with the following tests.

#### A. COVERING POWER

##### 1. Percent transmitted light

In determining the percent transmitted light,  $I_t$ , which

is a measure of white light transmitted by a fabric within the range of 1% to 20% transmission, a photoelectric cell, a light source, and a sample were arranged in a wooden box, the inside surface of which was painted a flat black. The amount of light transmitted through a circular area of each sample which was illuminated by diffused light was measured. A 100-watt frosted incandescent lamp placed six inches from the sample was used to illuminate the sample. The sample was hung in a vertical plane free from externally applied tension and was held against a two-inch diameter hole. A Weston photoelectric cell, model 594-RR, was placed in the beam of transmitted light, about eighteen inches from the sample, and a Simpson microammeter, model 29 (0-50 microampere range), was used to measure the output of the cell. The instrument was calibrated by adjusting a variable transformer which was connected between the instrument and a constant voltage transformer to give a meter reading of 36.6 milliamperes when a neutral filter having a transmission of approximately 12.5% is substituted for the fabric sample. Light transmission in percent as recorded in Table 1 was calculated by dividing the average of four meter readings for four samples by three.

##### 2. Percent reflected light, $I_r$

This test was performed in accordance with the measurements as described in U.S. Patent 2,828,528.

#### B. SOILING TEST

##### 1. Dry soil

The relative soilability of the woven fabric was tested by tumbling in the presence of a standard dry soil composed of the following materials:

|                      | Grams |
|----------------------|-------|
| Humus                | 35    |
| Cement               | 15    |
| Silica (60-200 mesh) | 15    |
| Clay (Kamec kaolin)  | 15    |
| Sodium chloride      | 5     |
| Carbon black         | 1.5   |
| Iron oxide           | 0.25  |
| Palmitic acid        | 1.6   |
| Oleic acid           | 1.6   |
| Coconut oil          | 3     |
| Lanolin (anhydrous)  | 1     |
| Kerosene             | 2     |
| Lauryl alcohol       | 0.5   |

The dry soil was mixed with 150 ml. of water, treated on a ball mill, dried at 110° C., and was then broken up and put through a 200-mesh screen.

The changes in reflectance after soiling and after washing expressed as percentage of the original reflectance were reported. The soiling-washing sequence was repeated twice. The reflectance measurements are the percent of the original reflectance, i.e., reflectance before soiling, retained after the washing following the second soiling.

Soiling was carried out by placing two samples in each of two jars of soil. The jars were tumbled with one hundred 0.25 inch stainless steel balls for forty-five minutes at 70° F. The reflectance of each sample was measured after soiling. The samples were then washed in a Launder-Ometer, manufactured by the Atlas Electric Devices Company, for twenty minutes in 200 ml. of distilled water at 100° F. with 0.25% of a detergent, made and sold by Procter and Gamble under the trade name "Tide," and fifty 0.25 inch stainless steel balls. After washing, the samples were rinsed in distilled water, air dried, and the reflectance again determined. Reflectance measurements were determined using a Photovolt reflectometer, model 610 (Photovolt Corporation). The instrument was calibrated using a white enamel working standard (catalog #6162, Photovolt Corporation) having 70-75 percentage reflectance with a green tristimulus filter (catalog #6130, Photovolt Corporation).

## 2. Oily soil

The procedure used in testing for resistance to oily soil is essentially the same as that described above for testing the resistance to dry soiling, except the soiling composition used is changed. The standard oil soil is composed of the following materials:

|                                                     | Grams |
|-----------------------------------------------------|-------|
| Coconut oil                                         | 1.2   |
| Peanut oil                                          | 1.2   |
| Cotton seed oil                                     | 1.2   |
| Lauric acid                                         | 0.4   |
| Myristic acid                                       | 0.4   |
| Palmitic acid                                       | 1.2   |
| Stearic acid                                        | 0.8   |
| Oleic acid                                          | 1.2   |
| Cholesterol                                         | 1.6   |
| "Primol D" (Standard Oil Co., N.J.)                 | 2.4   |
| "Oil-Dag" (Acheson Colloids Co., Port Huron, Mich.) | 15.0  |

The above materials are dispersed in 3200 ml. of carbon tetrachloride and the dispersion stirred well before using. The reflectance measurements reported in Table 1 are on the same basis as those described for the dry soil test.

## C. LUSTER HIGHLIGHT RATING

The luster highlight rating was determined by averaging the subjective ratings of six persons. Ratings were made on a scale from 1 to 5 with a rating of 1 representing no luster highlight and a rating of 5 representing a high luster highlight.

TABLE 1

|                                                              | Sample   |                |          |
|--------------------------------------------------------------|----------|----------------|----------|
|                                                              | F-1      | F-2<br>(Round) | F-3      |
| <b>Filament parameters:</b>                                  |          |                |          |
| Angle A (°)                                                  | 86       |                | 56       |
| M                                                            | 1.33     | 1.0            | 1.46     |
| $\frac{r_1}{R}$                                              | 0.27     |                | 0.48     |
| <b>Fabric Construction:</b>                                  |          |                |          |
| Ends and Picks                                               | 122 x 92 | 123 x 88       | 120 x 86 |
| Weight (Oz./Yd. <sup>2</sup> )                               | 1.99     | 1.96           | 2.00     |
| <b>Covering Power:</b>                                       |          |                |          |
| I <sub>s</sub> (percent)                                     | 5.4      | 6.0            | 4.8      |
| I <sub>r</sub> (percent)                                     | 75.8     | 65.5           | 78.6     |
| <b>Soiling Test (Percent Original Reflectance Retained):</b> |          |                |          |
| Dry Soil                                                     | 50.9     | 52.8           | 61.6     |
| Oily Soil                                                    | 75.1     | 67.9           | 76.7     |
| Luster Highlight Rating                                      | 4.25     | 1.25           | 3.08     |

The results of the tests show superior covering power for fabric sample F-1 which was prepared from the filaments of the present invention than for the round filament control sample F-2. Similarly, greater resistance to soiling was shown for sample F-1 than for sample F-2. The luster highlight for sample F-1 was much greater than for either the round sample F-2 or the trilobal sample F-3. It was also found that the trilobal sample F-3 exhibited an over-all surface sheen which was not apparent in sample F-1.

## EXAMPLE II

Continuous filaments of polyethylene terephthalate were melt spun at a temperature of about 285° C. from a spinneret containing ten orifices having the shape shown in Fig. 5 in which R<sub>1</sub> was 0.020 inch, R<sub>2</sub> was 0.015 inch, and R<sub>3</sub> was 0.001 inch. The polymer contained 0.3% by weight of titanium dioxide. The filaments were wound up in a bundle at a speed of 600 yards per minute and were subsequently drawn about 4.5 times their original length. After drawing, the filaments had a denier of about 15. The cross-sectional shape had the following parameters: Arm angle A=100°;

$$\text{Tip radius } \frac{r_1}{R} = 0.25$$

and modification ratio M=1.35.

- 5 A yarn having a total denier of about 900 was prepared by plying the filaments together. The yarn was then bulked as described in the copending application of Breen and Lauterbach, Serial No. 698,103, filed November 22, 1957. Three ends of the bulked yarn were then plied and twisted to give a total denier of approximately 3500. This yarn was then tufted into a loop pile carpet containing about 22 ounces of pile yarn per square yard of jute backing. A carpet of similar construction was prepared using round filaments.
- 10 In comparing the two carpet samples, a unique luster highlight was exhibited by the carpet prepared from the filaments of the present invention. The luster highlight was absent in the sample prepared from the round filaments. The resistance to soiling of the sample prepared from the fibers of the present invention was significantly better than that prepared from the round fibers.
- 15

## EXAMPLE III

A number of polymethyl methacrylate cylinders were machined to give enlarged fiber models having cross-sectional shapes defined by the parameters listed in Table 2. The models were rated subjectively by four persons for luster highlight with a rating of 1.0 representing no luster highlight and a rating of 7.5 representing a very high luster highlight. The data recorded in the table was the average of the four evaluations.

TABLE 2

| Sample No. | Arm Angle A° | $\frac{r_1}{R}$ | M    | Rating |
|------------|--------------|-----------------|------|--------|
| 1 (Round)  |              |                 |      |        |
| 2          | 80           | 0.52            | 1.19 | 5.0    |
| 3          | 96           | 0.5             | 1.22 | 4.0    |
| 4          | 80           | 0.4             | 1.25 | 6.5    |
| 5          | 80           | 0.3             | 1.32 | 5.0    |
| 6          | 80           | 0.2             | 1.39 | 4.5    |
| 7          | 90           | 0.1             | 1.53 | 3.0    |
| 8          | 80           | 0.1             | 1.45 | 3.0    |
| 9          | 108          | 0.1             | 1.39 | 6.0    |
| 10         | 108          | 0.3             | 1.28 | 7.5    |
| 11         | 118          |                 | 1.39 | 5.7    |
| 12         | 146          | 0.1             | 1.17 | 4.5    |
| 13         | 140          | 0.3             | 1.15 | 5.0    |
| 14         | 80           | 0.6             | 1.15 | 3.5    |
| 15         | 80           | 0.7             | 1.11 | 3.7    |

Another group of models having parameters outside the range of those of the present invention were prepared. The parameters and ratings for these models are set forth in Table 3 which follows.

TABLE 3

| Sample No. | Arm Angle A° | $\frac{r_1}{R}$ | M    | Rating |
|------------|--------------|-----------------|------|--------|
| 16         | 60           |                 | 2.0  | 2.0    |
| 17         | 80           |                 | 2.0  | 2.0    |
| 18         | 140          | 0.5             | 1.10 | 2.5    |
| 19         | 140          | 0.7             | 1.06 | 1.5    |
| 20         | 98           | 0.7             | 1.02 | 1.6    |
| 21         | 60           | 0.8             | 1.11 | 2.5    |
| 22         | 84           | 0.9             | 1.01 | 1.0    |
| 23         | 100          | 0.9             | 1.03 | 1.2    |
| 24         | 140          | 0.9             | 1.02 | 1.0    |
| 25         | 72           | 0.97            | 1.01 | 1.0    |

The foregoing examples illustrate the fact that the cross-sectional shape of the fibers or filaments of the present invention is critical in producing yarns and textile materials which have a combination of luster highlight, good covering power, soil resistance, and other desirable physical properties.

The filaments of this invention may be used to prepare either staple fibers or continuous filament yarn from a variety of synthetic polymers. Among the most important

polymers are the polyamides such as polyhexamethylene adipamide, polyhexamethylene sebacamide, polycaproamide, polyyxylene azelamide, polyoctamethylene oxalamide, polypyrrolidone, polymetaphenylene isophthalamide, polymetaphenylene adipamide; copolyamides, and irradiation grafted polyamides; the polyesters and copolymers such as the condensation products of ethylene glycol with terephthalic acid, ethylene glycol with a 98/2 mixture of terephthalic/5-(sodium sulfo)-isophthalic acids, ethylene glycol with a 90/10 mixture of terephthalic and isophthalic acids, polyesters derived from 2,2-bis(4-hydroxyphenyl) propane, and trans-p-hexahydroxyethylene glycol with terephthalic acid; acrylonitrile polymers and copolymers such as polyacrylonitrile, copolymers and terpolymers of acrylonitrile and vinyl pyridine, vinylidene chloride, vinyl chloride, or methyl acrylate; vinyl chloride polymers and copolymers, vinylidene chloride polymers and copolymers; polyurethanes, e.g., those described in French Patent 1,172,566, polyesteramides, polyethylenes, polypropylenes, especially linear polypropylene, polycarbonates such as those derived from 2,2-bis(4-hydroxyphenyl) propane, fluorinated ethylene polymers and copolymers such as polymers of tetrafluoroethylene hexafluoropropene, and monochlorotrifluoroethylene; composite filaments such as, for example, a sheath of polyamide around a core of polyester as described in the application of Breen, Serial No. 621,443, filed November 9, 1956, now abandoned, of which Serial No. 771,676, filed November 3, 1958, is a continuation-in-part, and two acrylonitrile polymers differing in ionizable group content spun as a sheath and core as described in the application of Taylor, Serial No. 640,722, filed February 18, 1957, now abandoned, of which Serial No. 771,677, filed November 3, 1958, is a continuation-in-part; cellulose derivatives such as cellulose acetate, regenerated cellulose, and the like. The fibers and filaments may be crimped or uncrimped, drawn or undrawn, bulked or unbalked, and twisted or untwisted. Mixtures of the above fibers as well as blends containing a major proportion of the synthetic fibers of this invention with a minor proportion of natural fibers or synthetic fibers of other cross sections may be used to prepare fabrics. The filaments may be spun in the form of two, monofilament yarn, multifilament yarn, roving, or the like.

The filaments of this invention are particularly useful in bulked form. Bulking may be conveniently achieved by a number of methods. For example, a particularly desirable bulking process is described in the copending application of Breen and Lauterbach, Serial No. 698,103, filed November 22, 1957. The novel filaments of this invention are peculiarly adaptable to being processed by the bulking process of the just mentioned application. The filaments of this invention may also be treated according to the process described in the copending application of Breen and Sussman, Serial No. 810,671, filed May 4, 1958, to provide desirable products.

Obviously slight variations in the configuration of the filaments of this invention may be present without impairing their desirable properties. Slight distortions may be introduced in the filament when it is spun or during the processing operations such as drawing, crimping, twisting, dyeing, bulking, and the like. Also, the filaments may contain small amounts of conventional additives such as dyes, pigments, titanium dioxide (up to about 2%), and the like.

The chief advantage of this invention is that it pro-

vides fibers, filaments, yarns, and fabrics having a unique combination of improved aesthetics and pleasing optical properties. In particular, it is possible, employing the fibers of the present invention, to prepare apparel fabrics having a combination of high resistance to wrinkling, good suppleness, flexibility and drapability, low soil pick-up, easy soil removal, high crush resistance, good light fastness, and good dye wash fastness. Fabrics possessing these improved properties may be achieved in addition to having a high degree of luster. It has not been possible using any prior art cross sections either round or non-round to produce apparel fabrics having this combination of improved properties.

The novel fibers and filaments of this invention may be employed to produce a wide variety of different types of woven, knitted, and non-woven fabrics, including both apparel and industrial textile products. Specific examples of these products include shirtings, suitings, dress and blouse fabrics, hosiery, sheeting, lingerie, taffetas, georgettes, sand-crepes, tissue-failles, foulards, broadcloths, batistes, rainwear, surah, tricot, tulles, circular knitted goods, satins, chiffons, sheers, wash-wear fabrics, crepes, casement fabrics, upholstery, carpets, filter cloths, ducks, beltings, webbing, braids, cordage and twine, fiber-reinforced laminates, tire cord, coated fabrics, pile fabrics, stuffing materials, floor coverings, tiles, batts, felts, furs, velvets, and the like.

As many widely different embodiments of this invention may be made without departing from the spirit and scope thereof, it is to be understood that this invention is not to be limited to the specific embodiments thereof except as defined in the appended claims.

I claim:

1. A textile filament prepared from a synthetic polymer, the cross section of said filament having three convex sides and three substantially symmetrical tip portions, said cross section having a tip radius ratio

$$\frac{r_1}{R}$$

and an arm angle A essentially within the range represented by the cross-hatched area on Figure 3 of the drawing, and a modification ratio M essentially within the range represented by the cross-hatched area on Figure 4 of the drawing.

2. The filament of claim 1 wherein said polymer is a polyester.

3. The filament of claim 1 wherein said polymer is polypropylene.

4. The filament of claim 1 wherein said polymer is a polyamide.

5. The filament of claim 1 in staple fiber form.

6. A textile yarn comprising the filaments of claim 1.

7. The yarn of claim 6 wherein said filaments are continuous filaments.

8. A textile fabric prepared from the filaments of claim 1.

#### References Cited in the file of this patent

#### UNITED STATES PATENTS

|           |                  |               |
|-----------|------------------|---------------|
| 414,090   | Taylor           | Oct. 29, 1889 |
| 1,773,969 | Dreyfus et al.   | Aug. 26, 1930 |
| 2,041,798 | Taylor           | May 26, 1936  |
| 2,373,392 | Hickey           | Apr. 17, 1945 |
| 2,831,748 | Finlayson et al. | Apr. 22, 1958 |

UNITED STATES PATENT OFFICE  
CERTIFICATE OF CORRECTION

Patent No. 2,939,202

June 7, 1960

Marlin C. Holland

It is hereby certified that error appears in the printed specification of the above numbered patent requiring correction and that the said Letters Patent should read as corrected below.

Column 8, line 26, for "ffoor" read -- floor --; line 44, strike out "by", second occurrence; line 65, for "2,373,392 Hickey" read -- 2,373,892 Hickey --.

Signed and sealed this 25th day of April 1961.

(SEAL)

Attest:

ERNEST W. SWIDER

Attesting Officer

DAVID L. LADD

Commissioner of Patents